

July 5, 1932.

C. R. MacDONALD

1,865,579

METHOD OF MANUFACTURING COMPOSITION ROOFING

Filed Aug. 9, 1928

2 Sheets-Sheet 1

Fig. 1.



Fig. 3.



Inventor

Chester R. Mac Donald

By *MacDonald*

Attorney

July 5, 1932.

C. R. MacDONALD

1,865,579

## METHOD OF MANUFACTURING COMPOSITION ROOFING

Filed Aug. 9. 1928

2 Sheets-Sheet 2



Inventor  
*Chester R. MacDonald*

By Macomber

Attorneys

## UNITED STATES PATENT OFFICE

CHESTER R. MACDONALD, OF MONROE, MICHIGAN, ASSIGNEE, BY MESNE ASSIGNMENTS,  
TO THE PATENT AND LICENSING CORPORATION, OF BOSTON, MASSACHUSETTS, A  
CORPORATION OF MASSACHUSETTS

## METHOD OF MANUFACTURING COMPOSITION ROOFING

Application filed August 9, 1928. Serial No. 298,515.

This invention relates to a method of manufacturing composition roofing.

An object of the invention is to provide a continuous process wherein a strip of fibrous material is first saturated with a low melting point asphalt or like material; coated with suitable material; slated, notched or slotted to define tabs and then, in a continuous manner, recoating the marginal portions of the strip while the strip is advancing in a horizontal plane, reslating such marginal portions, applying the same to pressure rolls or the like and finally longitudinally dividing the web to provide shingle strips of desirable character.

It is ordinarily the practice of roofing manufacturers to saturate, coat, and slate a web of material and to thereafter slot the same. It is advisable to recoat and reslate at least portions of the web containing the slots to the end that the complete shingle will be sightly in appearance and the notched portions thereof will be coated and slated to prevent deterioration thereof. My invention, therefore, contemplates these steps of resurfacing and recoating as a continuous process, while advancing the slotted web and maintaining it in a horizontal plane and applying to the marginal portions thereof an asphalt coating of suitable viscosity which gradually gravitates downwardly around the notched portions and marginal edges; thence slating such marginal portions of the advancing web, applying pressure thereto and finally longitudinally and transversely dividing the web to define shingle strips of desired configurations.

There are other subordinate objects of the invention which will be apparent to those skilled in the art from the reading of the following specifications in conjunction with the drawings attached hereto and forming a part hereof, in which—

Figure 1 represents in a schematic manner the preferred sequence of steps designated as A, B, C, D, E, and F;

Figure 2 represents in a like diagrammatic manner a sequence of steps preceding step C and designated A<sup>1</sup>, A<sup>2</sup>, A<sup>3</sup>, A<sup>4</sup>, A<sup>5</sup>, and A<sup>6</sup>, illustrating the idea of first slotting the roof-

ing felt and thereafter saturating, coating, slating and compressing it before its marginal portions are recoated and resurfaced, etc., as designated by steps C and D of Figure 1.

Figure 3 is a view of a pressure belt arrangement that may be used in lieu of or in conjunction with step E as shown in Figure 1.

In the manufacture of composition roofs, as aforesaid, it is the usual practice to first saturate and coat the web of felt before transversely slotting the same to form tabs. It, therefore, becomes necessary to recoat the slotted portions of the web and exposed edges and to reslate the same to the end that a durable shingle may be obtained and one which presents a pleasing appearance. In some instances, this recoating and resurfacing has been accomplished by hand dipping of individual strips by an operator taking one side portion of the strip and vertically submerging it into the coating medium and slating the same. This procedure obviously runs into a considerable item of expense. Such a vertical submersion of the strip furthermore applies the asphalt and coating to both the upper and lower surfaces of the shingle.

It will be apparent from the diagrammatic illustration contained in Figure 1 that my invention is based upon the discovery that such a recoating and resurfacing procedure may be carried out in a continuous manner without the necessity of hand manipulation and also without requiring that the web be vertically submerged in the resurfacing and reslating medium.

Referring particularly to Figure 1 of the drawings, 1 represents a web of felt or like roofing material which has previously been saturated with a low melting point asphalt or the like and has been coated in the manner known in the art by a suitable weatherproof coating and also surfaced with slate or similar comminuted mineral. This saturated, coated and slated web is thereafter slotted as shown at 2 to form tabs 3 in a manner well known in the art. The web thus slotted is thence continuously advanced to the point

55

65

70

75

80

85

90

95

100

denoted by step C in the drawings, at which point asphalt, the viscosity of which is regulated as desired, is applied to the marginal portions only as shown by reference character 4 leaving the intermediate central portion. 5 without the layer of recoating material. The viscosity of the asphalt is such that it will gravitate downwardly around the edges of the strip and slots therein without however running inwardly to the central zone of the strip, which zone is not desired to be recoated. Thus the asphalt is maintained in a rather viscous or heavy state so that it will not have a decided tendency to migrate inwardly towards the central portion of the web, but inasmuch as it is applied at the marginal edges it will naturally gravitate downwardly to coat the edges of the cut-outs. This recoating step occurs while the web is maintained in a horizontal plane and consequently the viscous asphalt gravitates downwardly so that it completely covers the edges of slots and margins of the web. If desired, a thin coating of asphalt may be applied to the under surface of the web but this is not essential. The thus recoated web is thereafter advanced, in a continuous manner, while maintaining it in a horizontal plane, to the point designated by step D in Figure 1 of the drawings where it is resurfaced with slate, mica, or other suitable materials or combinations of materials. This coating of slate is likewise applied only to the longitudinal marginal portions of the web, without slating the central portion thereof as shown by reference numeral 6. Reference numeral 7 designates the reslated longitudinal portions of the web. The web is thereafter continuously advanced to any suitable kind of pressure rolls as shown, for example, schematically in step E of Figure 1 wherein the recoated and resurfaced web is led between the rolls 8. As stated, the pressure belt arrangement shown in modification E', Figure 3, may be employed in lieu of or in conjunction with the bed pressure rolls shown in step E of Figure 1. This modification consists of an endless top pressure belt 8' and an endless bottom pressure belt 8'' between which the roofing web is fed.

After the web has been resurfaced, reslated and subjected to the pressure of rollers or belts, as aforesaid, the same is longitudinally divided, preferably during the course of its travel, slitting the same as at 9, and transversely dividing the same so that strips of suitable lengths and dimensions may be obtained.

It is also within the contemplation of this invention to slightly change the sequence of steps in accordance with the diagrammatic showing of Figure 2 wherein the felt A<sup>1</sup>, before saturation, is first slotted as at A<sup>2</sup> and thereafter saturated with a low melting point asphalt in any desirable manner as at A<sup>3</sup>;

coated at A<sup>4</sup>, slated at A<sup>5</sup>, conveyed over a festooning mechanism A<sup>6</sup>, after which the slotted web, thus coated and slated, is advanced while maintaining it in a horizontal plane to a position where asphalt is sprayed or otherwise applied on its marginal portions thereof as in step C of Figure 1; the marginal portions thereof thereafter slated as in step D of Figure 1; then subjecting the same to pressure rolls or pressure belts as in E of Figure 1 and finally slitting the same longitudinally as in F of Figure 1.

It will be apparent from the foregoing that my invention contemplates a continuous process of treating a roofing web in order to resurface and reslate the exposed marginal portions thereof at a minimum of expense and without the necessity of any hand manipulation or unnecessary wastage of materials. I realize however, that the particular steps or forms of apparatus herein disclosed and described are not entirely necessary to carry out my invention and that numerous changes in such procedure may be made without departing from the spirit of the invention as within the reasonable scope of the following claims:

Having thus described the invention, what I claim is:

1. A process of manufacturing composition shingles, the steps which comprise the saturation and slating of a web and thereafter the slotting thereof to define tabs and in continuously advancing the thus saturated and slotted web to a position for receiving a recoating of asphalt or like material thereon on the opposite upper marginal faces only thereof and in subsequently reslating at least the exposed tabs thereof and dividing the web into shingle strips of desired configuration and lengths.

2. A process of manufacturing composition shingles, which comprises the saturation and slotting of a web felt, coating the upper opposite marginal faces only of the web, including the notched portions and the edges of the web to seal the same, applying slate to such portions, and in finally dividing the same to provide shingle strips.

3. A continuous process of manufacturing composition shingles, which comprises the following steps; advancing a slotted web in a horizontal position, applying a viscous coating of asphalt to the opposite marginal faces thereof including the edges and on the upper surface thereof, reslating such marginal portions of the web only and in thereafter dividing the web into strip shingles.

4. A continuous process of manufacturing shingles consisting in feeding a slotted, saturated, coated and slated felted web, while maintaining it in a horizontal position, to a position where recoating of the longitudinal opposite marginal zones only thereof occurs, in thereafter slating such marginal zones only of the web and thereafter subdividing

the web to obtain shingle strips of desired sizes.

5. A continuous process of manufacturing shingles consisting in feeding a slotted and coated felted web, while maintaining it in a horizontal plane, to a position wherein its upper, opposite marginal portions only are coated by spraying asphalt thereto, in continuously advancing the web and slating such 10 marginal portions only thereof and in finally sub-dividing the web to obtain shingle strips of desired sizes.

6. The steps in the process of manufacturing shingles consisting in feeding a slotted shingle web in a horizontal plane, applying asphaltic material to the opposite marginal zones only of said web, but not to the intermediate or central zone thereof and in thereafter slitting said web to provide shingle 20 strips of desired sizes.

7. The steps in the process of manufacturing shingles consisting in continuously advancing a slotted web of roofing base while maintaining it in a horizontal plane, applying 25 comminuted minerals to the opposite marginal portions only of said web and in thereafter dividing said web to provide shingle strips of desired sizes.

8. A continuous process of manufacturing 30 composition shingles consisting in continuously advancing a slotted web while maintaining it in a horizontal plane, applying a coating of asphalt of a substantially non-spammable consistency to the opposite marginal 35 zones only of said web, but leaving the central portion thereof free from such coating, reslating the marginal portions of the web only as the same is continuously advancing in a horizontal plane, subjecting the thus recoated and reslated marginal portions of the web to pressure to firmly imbed the slate in the asphalt and in finally longitudinally slitting the web as it advances.

40 In testimony whereof I affix my signature.  
45 CHESTER R. MACDONALD.